

## UNITED STATES PATENT OFFICE

2,435,925

## REVERSE DETERGENT

Willard H. Kirkpatrick and Doyne L. Wilson,  
Sugar Land, Tex., assignors to Visco Products  
Company, Houston, Tex., a corporation of Dela-  
ware

No Drawing. Application November 22, 1944,  
Serial No. 564,713

2 Claims. (Cl. 252—161)

1

Our invention relates to the chemical purification of contaminated surfaces, and more specifically to the reconditioning of surfaces which have been contaminated with water or its chemical equivalent and which need to be substantially purged of traces of such contamination. For instance, metallic parts are often reduced to precisely finished shapes by machine tools while the temperature is kept down by a water containing coolant. Such a part, after air drying, even at elevated temperatures, in most instances will still retain a definite chemical contamination with water or other hydrophilic body, the presence of which can be ascertained by the fact that it is not readily wetted with oil. Another instance is the oil drums used to ship both lubricating and fuel oils. Especially when these are used for transoceanic shipment, after they have been emptied, they are likely to be seriously soiled or contaminated, both inside and outside. It is not uncommon to heat them with steam jets of very hot steam and to rinse them with caustic, either with or without a preliminary steam heating. In this way, it is possible to eliminate practically all the contamination except the residual water contamination left after the application of caustic or any other aqueous solution.

In many instances, such traces of water are more or less objectionable, sometimes to such an extent as to prevent further use of the container or to require lengthy and expensive reconditioning processes.

We have discovered that it is possible to treat such surfaces with a non-aqueous and hydrophobic liquid compatible with or frequently identical with the intended contents of the container or the rust-protecting preparation with which the machine part is to be coated, in which liquid is dissolved a percentage of a reagent dispersible or soluble in the liquid itself but also hydrophilic to such an extent that the chemical trace of water on the surface is taken into the applied liquid or rinse, so that the rinse can be poured off and leave the surface in a condition such that the hydrophobic material subsequently placed in contact with the container or machine part will readily wet it and find not even a chemical trace of water present at the contact surface.

In preparing one suitable reagent for the practice of the invention we employ the following ingredients:

1. Amyl naphthalene: A mixture of monoamyl- and diamyl-naphthalenes having the following specifications:

Sp. G. at 20° ..... 0.94-0.96  
M. W. ..... 231-56

Engler distillation by ASTM method D-86-35

2 modified as outlined in Sharples Standard Practice instructions.

- 1 cc. not below 250° C.  
95% between 250°-400° C.
- 5 2. Isopropanol: Regular 99% commercial grade.  
3. Sulfuric acid: Regular 98% commercial grade.  
4. Coumarone indene fraction: A distillate 10 fraction of coal tar commonly known as heavy solvent naphtha boiling between 160°-200° C. and having a minimum polymerizable content of 30% as determined by method of Ellis & Rabinowitz, described in Jour. Ind. Eng. Chem., 8, 797 (1916).  
15 5. Cyclohexylamine: Regular commercial grade.  
6. Ammonia: Regular 26° Bé commercial grade.  
7. Gas oil: Common commercial grade.  
20 8. To produce a reagent according to the invention, 2625 pounds of amylnaphthalene and 327 pounds of isopropanol are mixed and 4800 pounds of 98% sulfuric acid is added at a temperature not exceeding 45° C. Sulfonation is carried out 25 at a temperature of 50° to 55° C. by maintaining at this temperature for two hours to yield an alkylated naphthalene sulfonic acid. The free acid is then washed out by dumping the reaction product into cold water while cooling to keep the 30 temperature below 80° C. The amount of cold water used is such that the final wash water at room temperature should not be less than 38° Bé nor more than 41° Bé. About 4000 pounds of water will usually give a result within the limits 35 stated; 1200 pounds of a petroleum fraction which we designate gas oil and which is not much different than a high boiling kerosene is usually added in the washing process. This permits a more ready stratification of the two layers. After 40 settling overnight, the clear upper layer is recovered and amounts to about 5500 to 6000 pounds. A convenient way to do this is to drain off the wash water which constitutes the lower layer, leaving the upper layer in the process kettle. To this, 375 pounds of cyclohexylamine is added and the temperature is brought up to 110° C., whereby the basic amine reacts with the alkylated naphthalene sulfonic acid to reduce the acidity of the resultant molecule. At this point 1153 45 pounds of coumarone indene fraction is added and the temperature raised to 115° C. where it is maintained for two hours. Under such conditions the coumarone-indene fraction condenses with the partially amino-reacted alkylated naphthalene sulfonate to form a liquid modified coumarone-indene resin wherein the modifying group consists of an alkylated naphthalene sulfonate. After this lapse of time, the source of heat is removed from the kettle and the temperature is allowed to fall to about 105° C., and then 50 55 60

110 to 150 gallons of water are added and thoroughly stirred. The acid wash water is allowed to settle and discharged to waste and the residual acidity of the mass is neutralized to methyl orange alkalinity with 26° Bé. ammonia. This usually requires approximately 475 pounds of the ammonia. The ammonium sulfate solution is allowed to settle out and if necessary the product is brightened by heating to about 105° C. to remove any water present in suspension. This completes the product and it is now ready for packaging and in a batch of the size given amounts to about 6800 pounds.

The proportions of the different ingredients may be varied considerably. Without attempting to state definitely just what the extreme limits are, it is stated that, beginning with 2625 lbs. of amylnaphthalene, the isopropanol may be from 275 to 330 pounds. The sulfuric acid is present in excess and therefore the amount can be indefinite. The petroleum fraction may be between 1000 and 1400 pounds; the cyclohexylamine may be from 360 to 460 pounds; and the coumarone indene fraction from 1000 to 1200 pounds. The 150 gallons of water is merely wash water and therefore the amount is indefinite.

The final product disclosed herein has a specific gravity of 1.02. It is not injured by limited exposure to the atmosphere, but prolonged and extreme exposure will cause it to dry out much as varnish does. Small amounts of water will blend into the mass and do no harm, and large amounts will settle out after prolonged standing. It has a characteristic odor suggestive of coal tar products and is stable up to 130° C. It has a viscosity or "body" similar to a light lube oil.

The material is best prepared for actual use by dissolving it in suitable hydrocarbon solvent for ease in application and handling. Such solvents as benzene, toluene, unleaded gasoline, kerosene, naphtha, gas oil, fuel oil, Diesel oil, bunker oil, and various alcohols, ketones, chlorinated aliphatics, organic sulphides, and carbon tetrachloride may be employed.

The ratio of the reagent to solvent may vary from somewhat less than 1% to essentially 100% reagent, depending upon conditions. For instance, for the general rinsing of drums or containers, a 5% solution of the reagent in ordinary commercial unleaded gasoline functions very well, but if the containers to be treated are heavily

coated with water, a higher percentage is preferable so that the rinse will not be exhausted too quickly.

After an extended period of use, the rinse will merely become weak and when this occurs it can be set aside and a layer containing substantially 100 percent water together with only traces of reagent will accumulate at the bottom on standing and can be drained off. Similarly, where treatment is by dipping parts in a reservoir, the bottom of the vessel is best formed with a sump and a valve to drain the same and the accumulated water may be drained off from time to time without interrupting the use of the bath. Water thus drained off contains such small amounts of the reagent that the loss is negligible, and treatment to recover the reagent is not worth while.

Without further elaboration the foregoing will so fully explain our invention that others may readily adapt the same for use under various conditions of service.

We claim:

1. The method of conditioning surfaces for use under conditions such that traces of water constitute a contaminant, which comprises rinsing the surfaces with a non-aqueous rinse consisting of a non-aqueous hydrophobic organic solvent in which is dissolved an oil soluble amine salt of a coumarone-indene resin modified alkylated naphthalene sulfonate.
2. A rinse for removing hydrophilic contaminant from solid surfaces comprising essentially a non-aqueous hydrophobic organic solvent and an amine salt of a coumarone-indene resin modified alkylated naphthalene sulfonate dissolved in said solvent.

WILLARD H. KIRKPATRICK.  
DOYNE L. WILSON.

#### REFERENCES CITED

The following references are of record in the file of this patent:

#### UNITED STATES PATENTS

| 45 | Number    | Name                | Date           |
|----|-----------|---------------------|----------------|
|    | 2,262,926 | Edgar et al. _____  | Nov. 18, 1941  |
|    | 2,137,404 | Hollerer _____      | Nov. 24, 1938  |
|    | 2,130,668 | Gunther _____       | Sept. 20, 1938 |
|    | 2,206,589 | Wayne _____         | July 2, 1940   |
| 50 | 2,139,276 | Lenher et al. _____ | Dec. 6, 1938   |
|    | 2,055,588 | Pospiech _____      | Sept. 29, 1936 |